

## UNITED STATES PATENT OFFICE

2,588,514

## FERROUS ALLOYS

James P. Gill, Latrobe, Pa., assignor to Vanadium-Alloys Steel Company, Latrobe, Pa., a corporation of Pennsylvania

No Drawing. Application August 5, 1950,  
Serial No. 177,963

7 Claims. (Cl. 75—123)

1

This invention relates to a new and unusual alloy steel suitable for tools and dies and to a method of controlling the physical characteristics of hardness and toughness in the steel.

It is recognized that tools and dies which are subject to abrasive wearing at the surface and heavy shock must have a hard, wear-resistant surface backed up by a strong, tough core. Numerous attempts have been made to provide tool steels having these properties, but to my knowledge none has been successful. It is possible to make a steel which will have an intensely hard surface, but all of the prior art steels which have been so prepared have either become hardened to a depth which affects the strength and toughness of the core or the hard exterior layer is so thin that it will crack or shatter under pressure or shock.

It is an object of the present invention to provide an alloy steel which is capable of resisting both shock and surface wear.

Another object of the invention is to provide a method of controlling the thickness of the wear-resistant surface layer of an alloy steel.

In its broadest sense, the invention contemplates the addition of a combination of alloying metals to a high-carbon, high-tungsten steel in an amount sufficient to result in hardening an exterior surface layer without hardening or affecting the strength of the core.

High-carbon, high-tungsten steels were among the earliest alloy tool steels. Steels containing high percentages of carbon and tungsten along with small percentages of other metals such as manganese were known to have a hard surface but it was determined that this hardness extended throughout the cross sectional dimension of the steel bar. These hard, brittle steels were adequate for certain purposes, such as for tools, lathes, planers and the like, which were designed for heavy cuts wherein shock resistance was not an important feature. These brittle steels were not satisfactory for use in tools and dies which were subject to impact, pressure or shock.

I have now discovered an alloy tool steel having certain definite concentrations of alloying elements as will be set forth in detail hereinafter. These steels will have a tough shock resistant core and a hard wear-resistant surface layer which is not subject to chipping or shattering. I have also discovered that I can vary the thickness of the hardened exterior layer by varying the amount of alloying elements in the steel.

The following examples illustrate the various steels which I have prepared in the practice of

the present invention along with an explanation of the best reasons available to me for the action of the various steels. It should be understood that I do not wish to be limited to any particular theory since the art of alloy steels is extremely complex and open to controversy. In each of the following examples the concentrations are given in percentages by weight unless otherwise specified.

10

## Example I

A steel was prepared by melting together iron suitable for use in tool steels along with the following alloying elements:

15

|             | Per cent |
|-------------|----------|
| Silicon     | .25      |
| Manganese   | .30      |
| Chromium    | .38      |
| Carbon      | 1.91     |
| 20 Tungsten | 10.19    |

20

and traces of impurities. Samples 1½" in diameter and 4" long of this heat were quenched at 1600° F. The samples were found to have an intensely hard surface layer which penetrated approximately  $\frac{3}{4}$  of an inch. Such a hardness penetration is desirable in a steel which must have exceptional resistance to wear and, at the same time, withstand heavy shock and high pressures.

30

## Example II

A heat was prepared by melting a suitable iron along with the following alloying elements:

35

|           | Per cent |
|-----------|----------|
| Silicon   | .24      |
| Manganese | .28      |
| Chromium  | .32      |
| Vanadium  | 1.03     |
| 40 Carbon | 2.02     |
| Tungsten  | 10.71    |

40

and traces of the usual impurities. Samples of this steel were quenched as in Example I and were found to have a comparable hardness penetration. The element vanadium did not materially change the hardening characteristics of the composition.

45

It was found that molybdenum could be substituted for the silicon, manganese or chromium in either Example I or Example II without materially affecting the hardening characteristics of the samples.

## Example III

A high carbon, high tungsten heat was pre-

55

pared using a suitable iron and alloying elements in the following proportions:

|                 | Per cent      |
|-----------------|---------------|
| Silicon -----   | .27           |
| Manganese ----- | .27           |
| Carbon -----    | 1.65 to 2.50  |
| Tungsten -----  | 7.50 to 15.00 |

When samples of this steel were quenched and tested, they were found to have a hard layer that was very thin, i. e.,  $1/64$  to  $3/64$  of an inch. Such a thin hardened surface layer will not withstand heavy shock or pressure.

#### Example IV

A heat was prepared employing suitable iron and alloying elements in the following proportions:

|                 | Per cent |
|-----------------|----------|
| Silicon -----   | .34      |
| Manganese ----- | 1.48     |
| Carbon -----    | 2.19     |
| Tungsten -----  | 10.37    |

When samples of this steel were quenched and tested, they were found to be extremely hard, but the hardness extended all the way through the  $1\frac{1}{2}$ " samples. Such a steel is typical of the older type tool steels which are unsuitable for use where they are subjected to shock and pressure.

Other heats and tests were made which have led me to conclude that the novel and unusual properties of my tool steel can be achieved only by carefully following the method outlined herein and limiting the amounts of alloying elements as will be hereinafter described.

In general it may be stated that my new alloy steel is an improved forgeable and machinable alloy steel containing iron and the usual impurities and from 1.65% to 2.50% carbon, from 7.50% to 15.00% tungsten, from 0 to 2.50% vanadium and not more than 1.50% of a combination of at least three alloying elements from the group consisting of silicon, manganese, chromium and molybdenum and the balance iron and the normal impurities of sulfur and phosphorus. The silicon, manganese, chromium and molybdenum may be individually present in amounts between 10% and 1.00%. A steel prepared according to the formula outlined above will be found to have a tough, ductile, shock-resistant core and a hard, wear-resistant surface layer which will be at least  $5/64$  of an inch in thickness and may be of a greater thickness which will not affect the toughness and softness of the core.

The thickness of the hardened surface layer can be adjusted and controlled by adjusting the amount of alloying elements which are added to the steel. For example, if the amount of silicon, chromium, manganese and molybdenum is maintained below 1.00% (as in Example I) a certain thickness is achieved. If the amount is increased nearly to 1.50%, the hardened surface layer will be thicker.

In order to illustrate the physical characteristics of a steel prepared according to the invention, but without intending to limit the invention in any way, it may be stated that the hardness of the surface layer is approximately 64 to 68 on the Rockwell "C" scale. The hardness of the core of the specimens prepared according to Examples I and II was approximately 47 on the Rockwell "C" scale. On the other hand, the surface hardness of the samples prepared ac-

ording to Example IV was 64 on the Rockwell "C" scale and a center hardness of 61 on the scale. It will be seen that this steel was approximately the same hardness all the way through and did not have a tough core. The steel made according to Example III had the same hard surface and soft core as the steels made according to Examples I and II but the hard layer was very thin and penetrated an insufficient depth of about  $1/64$  to  $3/64$  of an inch.

This application is a continuation in part of my copending application Serial No. 750,837, filed May 27, 1947, now abandoned, which was a continuation in part of my then copending application Serial No. 659,878, filed April 5, 1946, now abandoned.

The invention is hereby claimed as follows:

1. An improved forgeable and machinable quenched alloy steel consisting essentially of about 1.65% to about 2.50% carbon, about 7.50% to about 15.00% tungsten, from 0% to 2.50% vanadium, an amount not exceeding 1.50% of a combination of at least three alloying elements from the group consisting of silicon, manganese, chromium and molybdenum and the balance iron and the normal impurities of sulfur and phosphorus, said alloying elements being individually present in amounts between 0.10% and 1.00%.
2. An improved forgeable and machinable quenched alloy steel consisting essentially of about 1.65% to about 2.50% carbon, about 7.50% to about 15.00% tungsten, from 0% to 2.50% vanadium and an amount not exceeding 1.50% of a combination of at least three alloying elements from the group consisting of silicon, manganese, chromium and molybdenum and the balance iron and the normal impurities of sulfur and phosphorus, said alloying elements being individually present in amounts between 0.10% and 1.00%, said amount being adjusted to cause hardening from the surface to a depth of about  $\frac{1}{64}$ ths of an inch across the section of a round bar  $1\frac{1}{2}$  inches in diameter or larger.
3. An improved forgeable and machinable quenched alloy steel consisting essentially of about 1.65% to about 2.50% carbon, about 7.50% to about 15.00% tungsten, from 0% to 2.50% vanadium, about 0.25% silicon, about 0.30% manganese and about 0.38% chromium and the balance iron and the normal impurities of sulfur and phosphorus.

4. A method of making an improved forgeable and machinable alloy steel which comprises melting together about 1.65% to about 2.50% carbon, about 7.50% to about 15.00% tungsten, from 0% to 2.50% vanadium, an amount not exceeding 1.50% of a combination of at least three alloying elements from the group consisting of silicon, manganese, chromium and molybdenum and the balance iron and the normal impurities of sulfur and phosphorus, said alloying elements being individually present in amounts between 0.10% and 1.00% and quenching said steel.

5. A method of making an improved forgeable and machinable alloy steel which comprises melting together about 1.65% to about 2.50% carbon, about 7.50% to about 15.00% tungsten, from 0% to 2.50% vanadium, an amount not exceeding 1.50% of a combination of at least three alloying elements from the group consisting of silicon, manganese, chromium and molybdenum and the balance iron and the normal impurities of sulfur and phosphorus, said alloying elements being individually present in amounts between 0.10% and 1.00% and heating and quenching said

steel, said amount being effective to cause hardening from the surface to about  $\frac{1}{64}$  of an inch across the section of a round bar about  $1\frac{1}{2}$  inches in diameter or larger.

6. A method of adjusting and controlling the thickness of a hardened surface layer in an alloy steel having a carbon content of about 1.65% to about 2.50% and a tungsten content of about 7.50% to about 15.00%, which comprises essentially incorporating into said steel while molten an amount not exceeding 1.50% by weight of a combination of at least three alloying elements from the group consisting of silicon, manganese, chromium and molybdenum, said alloying elements being individually present in amounts between 0.10% and 1.00% and quenching said steel.

7. A method of adjusting and controlling the thickness of a hardened surface layer in an al-

loy steel having a carbon content of about 1.65% to about 2.50% and a tungsten content of about 7.50% to about 15.00%, which comprises essentially incorporating into said steel while molten about 0.25% silicon, about 0.30% manganese and about 0.38% chromium and quenching said steel.

JAMES P. GILL.

#### REFERENCES CITED

The following references are of record in the file of this patent:

Alloys of Iron and Tungsten, pages 159 to 160. Edited by Gregg. Published in 1934 by the McGraw-Hill Book Co., New York, N. Y.

Tool Steel Simplified, page 46. Edited by Palmer. Published in 1937 by the Carpenter Steel Company, Reading, Pa.